

# UNITED STATES PATENT OFFICE.

GERSHOM MOORE PETERS, OF CINCINNATI, AND MILTON FLETCHER LINDSLEY, OF KINGS MILLS, OHIO, ASSIGNEES TO THE KING POWDER COMPANY, OF CINCINNATI, OHIO, A CORPORATION OF OHIO.

## EXPLOSIVE.

977,545.

Specification of Letters Patent.

Patented Dec. 6, 1910.

No Drawing. Application filed December 6, 1907, Serial No. 405,362. Renewed October 20, 1910. Serial No. 588,183.

*To all whom it may concern:*

Be it known that we, GERSHOM MOORE PETERS, a citizen of the United States, residing at Cincinnati, in the county of Hamilton and State of Ohio, and MILTON FLETCHER LINDSLEY, a citizen of the United States, residing at Kings Mills, in the county of Warren and State of Ohio, have invented certain new and useful Improvements in Explosives, of which the following is a full, clear, and exact specification.

This invention relates more particularly to explosives for blasting purposes, and of this class it has especial reference to the species required in mining operations.

The dangers to life from firing blasts in mines where explosive gases accumulate have caused the enactment of laws in many localities, prohibiting the use of blasting powders which emit flame or generate sufficient heat when fired to ignite these gases. Many attempts have been made to produce an explosive free from these defects, but as a rule they are open to three main objections which exclude them from general use, viz. they are too expensive to manufacture, they produce too much smoke and offensive gas, or they have to be fired by a detonating cap to the use of which the average miner is not accustomed and is greatly opposed.

This invention aims to avoid these objections and therefore has for its primary object to produce an explosive capable of being used like ordinary black blasting powder and other similar forms of explosives, but which will possess in the required degree the necessary qualities of being free from objectionable flame and heat, and will at the same time be reasonable in cost of production.

A further object of the invention is to produce an explosive especially adapted for mine blasting purposes, which, when ignited, will generate an excessive volume of steam, which will not only dampen down the heat and flame, but will slow down the action of the blast and materially increase the heaving power of the explosion.

With a view to the attainment of these ends and the accomplishment of certain other objects which will hereinafter appear, the invention consists of an explosive possessing certain novel characteristics which

will first be specifically described, and then more generically pointed out in the claims. 55

In carrying out the invention, we employ an explosive agent or ingredient which explodes at a comparatively low temperature and gives off an excess of hydrogen gas which, when united with oxygen, instantly 60 produces a large volume of steam, effectively reducing and dampening down the heat, flame and smoke that would naturally be caused by the other ingredients of the compound. The presence of this excess of 65 steam at the instant of explosion produces not only these desirable qualities, but the further important function of slowing down the action and hence materially increasing the heaving power of the explosion, which is 70 very desirable in a blasting powder, especially in coal mining operations, as this slow action and increased heaving power has the desired effect of loosening and throwing down the coal without shattering it into 75 small bits, as is the case where the explosive has a more rapid action. In combination with this steam producing element, we employ nitrate of soda, whose explosive strength is greatly enhanced by the hydrogen gas, and to these three elements should be added carbon in sufficient quantity to 80 support combustion.

As an element or agent possessing in a marked degree the qualities of the first ingredient before named, we employ nitrate of ammonia. In case this should not be pure, however, there might develop some free acid, which, under some conditions, might render the explosive not altogether 90 safe. To guard against the presence of such acid, we add to the compound a suitable neutralizing agent, such as carbonate of calcium, carbonate of magnesia, or carbonate of soda, but preferably the carbonate of calcium, which is less expensive than either of the others, and is much more effective, as well as less hygroscopic than carbonate of soda, and is better adapted for the purpose than carbonate of magnesia, as it possesses 100 greater specific gravity and is less bulky.

The nitrate of ammonia and nitrate of soda employed in the compound are hygroscopic, and of course this condition in an explosive is to be avoided. For that reason, 105 therefore, we add to the compound consist-

ing of the foregoing elements, a suitable agent which will destroy to the necessary degree the power of these two elements to attract moisture. As an ingredient best suited for this purpose we employ brimstone. The formula, therefore, which we have found to be most efficient, and which will carry out in a maximum degree the principles of this invention, consists of the following ingredients, employed in substantially the proportions set opposite each, *i. e.*—

|    |                           |      |
|----|---------------------------|------|
| 15 | Nitrate of soda-----      | 48%  |
|    | Nitrate of ammonia-----   | 24%  |
|    | Carbonate of calcium----- | 4%   |
|    | Brimstone -----           | 12%  |
|    | Charcoal-----             | 12%  |
| 20 | Total -----               | 100% |

The process of combining, mixing and preparing these ingredients does not, or need not, differ from the well known process of making ordinary black blasting powder, the ingredients being mixed, incorporated, pressed, granulated, dried, glazed, sifted and packed in the same or any approved way.

The described formula is inexpensive and can be safely manufactured, stored and transported. It can also be granulated to suit different kinds of blasting operations or different kinds of coal to be mined, and is especially adapted for coal mining operations, inasmuch as it may be fired by means of a fuse in the ordinary method with which miners are familiar. The initial cost may be somewhat more than that of common black blasting powder, but it has greater strength per given quantity, and will not shatter and destroy the coal to the same ex-

tent, and it may therefore be said is more economical, as has been demonstrated by actual tests. In addition to these desirable qualities, this explosive possesses the further important quality of being sufficiently free from flame and heat to avoid the danger from the presence of explosive gases lurking in the mines, and it is almost entirely devoid of smoke and odor and consequently the miners are enabled to start in at once to remove the coal thrown down without waiting for these objectionable fumes to subside.

In order that the invention may be understood and used by those skilled in the art, an example of a formula for carrying out the invention and the particular proportions which have been found best adapted for the accomplishment of its objects have been thus specifically described, without, however, any intention of limiting ourselves thereto, for

What we claim is:

1. An explosive compound consisting of a mixture of nitrate of soda, nitrate of ammonia, carbonate of calcium, brimstone, and charcoal.

2. An explosive compound containing nitrate of soda, about 48%, nitrate of ammonia, about 24%, carbonate of calcium, about 4%, brimstone, about 12%, charcoal, about 12%.

In testimony whereof we have signed our names to this specification, in the presence of two subscribing witnesses, on this 2nd day of December A. D. 1907.

GERSHOM MOORE PETERS.  
MILTON FLETCHER LINDSLEY.

Witnesses:

A. M. BECKLEY,  
E. R. MERCKEL.